

## UNITED STATES PATENT OFFICE

2,512,441

## CORE AND MOLDING SANDS

Lucien Rouzet, Clichy, France, assignor to  
 "L'Impregnation," Clichy, France

No Drawing. Application September 5, 1946, Serial No. 695,045. In France January 24, 1940

Section 1, Public Law 690, August 8, 1946  
 Patent expires January 24, 1960

2 Claims. (Cl. 22—188)

1

It is highly desirable in foundry work to agglomerate the core and molding sands by means of an agglomerating agent which on the one hand is completely consumed by the heat of the molten metal, to allow the sand to come out after cooling, and which on the other hand at the temperature of the molten metal is sufficiently plastic to yield to the shrinkage of the metal during its cooling.

The agglomerates at present used in founding do not possess this thermo-plasticity or only possess it to an insufficient extent. This results in flaws, which are the cause of considerable wastage.

These disadvantages are avoided according to the invention, owing to the fact that a synthetic resin is used as agglomerant.

A synthetic resin with a basis of amylose material is preferably utilized, of the type described in the specification of our co-pending patent application No. 695,044 entitled "Improvements relating to synthetic resins."

As described in the said specification, the preparation of this new synthetic resin may, for example, be carried out in the following fashion:

1 kg. of soluble starch is dissolved in 2 liters of 40% formaldehyde. This solution is neutralized, and is heated to 100° centigrade and kept at this temperature for two hours. The solution has then become clear and very fluid. To this solution is added:

200 grams of urea;  
 75 grams of phenol;  
 20 grams of carbonate of soda.

The temperature is maintained at 100° for another 15 minutes and then cooling takes place. In this way a coloured liquid is obtained, which is soluble in water and in mineral and vegetable oils, but which precipitates in alcohol.

The liquid product thus obtained may be dried in a vacuum, and is then obtained in the form of a hard, translucent material, difficult to crush, and appearing as a true resin.

This synthetic resin is utilized as an agglomerant either in solid form or in a more or less syrupy or pasty state.

To prepare the core sand or molding sand according to the invention, it is possible according to a first example to treat the sand with a quantity of 3 to 5% of the said synthetic resin.

According to another example an agglomerant is prepared consisting of a mixture of: 75 kg. of the said amylose synthetic resin, 23 kg. of siccative oil, and 2 kg. of non-siccative oil; and the sand will be treated with a quantity of from 2 to 3% of this agglomerant.

2

The procedure will be similar in the case of other synthetic resins such as vinylic resins and the like.

The sands and cores prepared with these agglomerants have the advantage that the agglomerant is completely consumed, whilst providing the requisite thermo-plasticity, so that the castings produced are free from flaws.

More especially the agglomerant with a synthetic amylose resin base has the advantage of a low cost.

As in the case of the second example mentioned above, the synthetic resin can be used dissolved in oil.

Naturally the examples indicated above are only given by way of example. The proportions as well as the ingredients mixed with the synthetic resin may vary according to the problems to be solved; cores may be packed by compressed air, by hand, striped on plates, in chills etc.

I claim:

1. A foundry composition comprising a body of sand and from 2-5% of a binder consisting essentially of a synthetic amylose urea phenol formaldehyde resin comprised of substantially more than one half starch, a major portion of the remainder being formaldehyde, with a smaller amount of urea and a still smaller amount of phenol.

2. A foundry composition comprising a body of sand and from 2-3% of a binder, the major fraction of which binder consists of a synthetic amylose urea phenol formaldehyde resin comprised of substantially more than one half starch, a major portion of the remainder being formaldehyde, with a smaller amount of urea and a still smaller amount of phenol, the remainder of said binder consisting substantially of a siccative oil.

LUCIEN ROUZET.

40

## REFERENCES CITED

The following references are of record in the file of this patent:

## UNITED STATES PATENTS

| Number       | Name   | Date          |
|--------------|--------|---------------|
| 2,121,076    | Ellis  | June 21, 1938 |
| 2,148,642    | Ricard | Feb. 28, 1939 |
| 2,203,471    | Ray    | June 4, 1940  |
| 50 2,212,314 | Bauer  | Aug. 20, 1940 |
| 2,246,635    | Moller | June 24, 1941 |

## FOREIGN PATENTS

| Number     | Country       | Date          |
|------------|---------------|---------------|
| 55 371,789 | Great Britain | Apr. 28, 1932 |
| 506,770    | Great Britain | June 5, 1939  |
| 515,470    | Great Britain | Dec. 6, 1939  |